

Patented Nov. 22, 1927.

1,650,541

## UNITED STATES PATENT OFFICE.

JOSEPH SCHÄFER, OF HALTINGEN, GERMANY, ASSIGNOR TO THE FIRM J. R. GEIGY  
S. A.

### TANNING ANIMAL HIDES.

No Drawing. Application filed September 1, 1926, Serial No. 133,087, and in Germany August 5, 1925.

The salts of hydrofluosilicic acid have been found to have a distinct action on animal hides prepared for tanning, and to produce a weak tanning effect; with these agents alone, however, it is not possible to obtain a leather suitable for placing on the market.

By the present invention, the hides are treated with a salt of hydrofluosilicic acid, prior to, or simultaneously with, a vegetable, mineral or synthetic tanning agent, such as, for example, a sulphite extract of quebracho, alum, a basic salt of chromium, iron or aluminium, tannin, or sulphite liquor, or with a mixture of such tanning agents.

When hides which have been treated with a salt of hydrofluosilicic acid, are tanned by means of the aforesaid tanning agents, the tanning agent is taken up extremely rapidly and easily, and in the correct quantity; and an excellent and uniform tanning effect is produced; the tanning is more complete, and occupies a shorter time than is the case in the usual tanning processes.

Another considerable advantage lies in the fact that the treatment with a salt of hydrofluosilicic acid produces a marked brightening effect in the tanned leather, some kind of bleaching action occurring as a result of the treatment.

A further advantage lies in the abundant absorption of the tanning agent which is

shown by hides which have been pre-treated with a salt of hydrofluosilicic acid.

Like results are attained if the treatment with the aforesaid salts occurs simultaneously with the treatment of the hides with the tanning agent.

To illustrate the rapidity in tanning attainable by the invention, it may be mentioned that after a pre-treatment with a hydrofluosilicate, sheep skins or small goat-skins may be tanned through, for example with a vegetable tanning agent, in about 3 hours, and calf-skins in about 6 hours, whilst if the pre-treatment is omitted, the remaining conditions being the same, a considerably longer time is necessary; for example, sheep-skins may require 2-3 days tanning, and calf-skins 2-4 days or more.

What I claim is:—

1. A process for tanning animal hides, comprising treating the same with a salt of hydrofluosilicic acid.

2. A process for tanning animal hides, consisting in treating the same previously with a salt of hydrofluosilicic acid and subjecting them thereupon to the tanning operation.

In witness whereof I have hereunto signed my name this 19th day of August, 1926.

JOSEPH SCHÄFER.